

April 29, 1924.

1,491,863

T. A. JANNEY

FLOTATION PROCESS

Filed Oct. 21, 1920



WITNESS:

*C. Burnap*

INVENTOR:

*Thomas A. Janney*  
BY

*Sheridan Jones, Sheridan & Smith, ATTORNEYS*

## UNITED STATES PATENT OFFICE.

THOMAS A. JANNEY, OF GARFIELD, UTAH.

## FLOTATION PROCESS.

Application filed October 21, 1920. Serial No. 418,466.

*To all whom it may concern.*

Be it known that I, THOMAS A. JANNEY, a citizen of the United States, residing at Garfield, in the county of Salt Lake and State of Utah, have invented certain new and useful Improvements in Flotation Processes, of which the following is a specification.

This application is a continuation in part 10 of my prior application Serial No. 262,812, filed November 16, 1918.

This invention relates to improvements in the concentration of mineral-bearing ores by the flotation process and to improvements in 15 oils for use in said process, which is now usually performed by subjecting the wet ore pulp to sub-aeration or to agitation in contact with air after adding to the pulp a small quantity of oil or other suitable frothing agent, sometimes with the further addition of sulphuric acid or other acid, whereby a mineral-bearing froth is formed which may be floated off or otherwise separated from the mixture.

20 My invention is based on the discovery that if coal tar or wood oils are used in the flotation process better metallurgical results will be obtained if such oils are reconstructed with sodium sulphide ( $Na_2S$ ) or other suitable reagents, whereby the oils are rendered more easily emulsifiable. I have found that the action of the oil as a metalliferous selective agent is further improved by reconstructing it with sulphur, as hereinafter described. The invention is particularly applicable to wood oils and to oils of crude coal tar, or a combination of both. For example, the present output of wood oils and certain oils of crude coal tar, are not easily emulsifiable and fail to give satisfactory results in the flotation process. It has been found that these oils may be reconstructed with certain reagents as hereinafter described, whereby they are put in such a state 25 that they are very easily emulsified and give results which are far superior to the results obtained with oil not so treated.

In carrying out the process, I prefer to use the apparatus illustrated in the drawings, although it will be understood that various other forms of apparatus may be used

in carrying out the process of reconstructing the oil. This apparatus comprises a tank 10 mounted above a furnace 11 having a fire box 12 and a grate 13. The oil to be treated is placed in this tank through an oil charging valve 14, and the tank is provided with another inlet opening 14<sup>a</sup> through which sodium sulphide or other reconstructing reagent is introduced into the tank. A plurality of condensing pipes 15 are connected to the upper part of the tank 10 and are inclined upwardly and rearwardly therefrom as illustrated, being surrounded through a part of their length by the water-jacket tubes 16 through which a circulation of cold water is maintained in order to effect the condensation of the contents of the tubes 15. The water is introduced to the water-jacket through the supply pipe 17 and causes the oil in the condensing pipes to condense and flow back into the tank 10 for further treatment. A safety valve 18 set preferably for five pounds pressure is connected to the upper part of the tank. In the reflux still or condenser, certain parts of the contents of the tank which will vaporize at the temperature to which it is subjected, are alternately vaporized and condensed until a thorough union of the oil and the sodium sulphide or other reagent is effected.

In reconstructing the oil by means of the process herein described, from one to four per cent by weight of sodium sulphide ( $Na_2S$ ) relative to the weight of the oil is introduced into the tank with the oil. A fire is maintained in the furnace beneath the tank in order to heat the mixture therein to a sufficient temperature to cause the agent and the oil to unite; that part of the oil which vaporizes rises in the tubes 15, is condensed therein, and then returns to the tank. This boiling of the mixture of oil and sodium sulphide is preferably carried on at a temperature of from 275° F. to 300° F., and is continued for a period of about one hour and a half or until the contents of the tank are homogeneous and uniform in character. The reconstructed oil so formed may then be drawn off through the pipe 20 to a suitable storage tank or reservoir.

I have found, however, that the quality of

the oil used in the flotation process may be further improved by boiling the same in the presence of sulphur, and if it is desired to give the oil this further treatment, the oil 5 after treatment with sodium sulphide is retained in the tank 10 and preferably allowed to cool, after which five per cent by weight of sulphur relative to the weight of the contents of the tank is introduced into the tank, 10 preferably in the form of flowers of sulphur. The mixture in the tank is then boiled again at a temperature of from 275° F. to 300° F. for a period of three or four hours. The resulting product is then drawn off and stored 15 for use in the flotation process. The temperature and duration of each treatment may vary somewhat depending on the oil being treated and upon the reagent used.

It is found that the reconstructed oil 20 formed by this double treatment gives very good results when used in the flotation process. For example, I have found that in treating copper ore by the flotation process with an untreated coal tar oil, the resulting tailing 25 contained .480% of copper, whereas, in another test operation on the same ore under the said conditions with the same oil after it had been reconstructed with sodium sulphide and sulphur, the resulting tailing 30 contained only .155% of copper, showing that the oil after being treated with sodium sulphide and sulphur is far superior as a metalliferous selective agent to the oil which has not been so treated.

35 It will be understood that the oil may be used after treatment with sodium sulphide alone, but, in general, it has been found that the results are further improved by further treatment of the oil with flowers of sulphur.

40 While the operations of treating the oil with sodium sulphide and flowers of sulphur may preferably be carried on successively, it is found that equally satisfactory results for flotation purposes may be obtained by treating 45 the oil with these two compounds or reagents simultaneously. In addition to sodium sulphide, it is possible to use sulphides of potassium, calcium, and various other sulphides of the alkali metals and the alkaline

50 earths. The oil after treatment with sodium sulphide or after treatment with both sodium sulphide and sulphur, as herein described, is ready for use in concentrating ore by the flotation process which may be carried out, 55 for example, by mixing the finely crushed ore with water to form a freely flowing pulp, adding a small quantity of the reconstructed oil, and in some cases a small quantity of sulphuric acid  $H_2SO_4$ , agitating the mixture of oil and pulp in contact with air to

60 form a froth and then separating the froth, as will be apparent to those skilled in the art. By treating the oil with sodium sulphide it is made alkaline and more easily 65 emulsified, whereby the invention is of par-

ticular advantage as a treatment for coal tar oils and other oils which give an acid reaction before being subjected to my improved process. The results obtained in the flotation process are particularly improved 70 when an alkaline coal tar oil is used.

Although I have described a particular method of carrying out my improved process for purposes of illustration, it will be understood that it may be performed in various ways without departing from the scope of the appended claims.

I claim:

1. The process of concentrating ores by flotation, which comprises adding to a wet 80 ore pulp a quantity of coal tar oil which has been boiled with an alkaline sulphide, and subjecting the mixture to a froth forming operation.

2. The process of concentrating ores by 85 flotation, which comprises adding to a wet ore pulp a quantity of an acid coal tar oil which has been boiled with sodium sulphide to form a union therewith, and then subjecting the mixture to a flotation operation.

90 3. The process of concentrating ores, which comprises adding to the wet ore pulp a coal tar oil frothing agent having normally an acid reaction which has been rendered alkaline by distillation in the presence of an alkaline sulphide, and subjecting the resulting mixture to agitation and aeration to form a mineral bearing froth.

95 4. The process of concentrating ores by flotation, which comprises agitating and 100 aerating the ore pulp with a quantity of coal tar oil which has been rendered alkaline by boiling in the presence of sodium sulphide.

5. The process of concentrating ores by flotation, which comprises agitating and 105 aerating the ore pulp with a quantity of coal tar oil which has been heated in the presence of sodium sulphide and sulphur.

6. The process of concentrating ores by flotation, which comprises agitating and 110 aerating the ore pulp with a frothing agent comprising a coal tar oil which has first been heated in the presence of sodium sulphide, and then heated in the presence of sulphur.

115 7. The process of concentrating ores by flotation, which comprises the operations of subjecting to a froth forming operation a wet ore pulp after adding to said pulp a small quantity of reconstructed coal tar oil which has been formed by boiling an acid oil in the presence of sodium sulphide at a temperature sufficient to vaporize the oil while condensing the vapors of distillation, and returning the distillates to the mixture during the boiling operation.

120 8. The process of concentrating ores by flotation, which comprises subjecting to a froth forming operation a wet ore pulp after adding to said pulp a quantity of coal tar oil which has been treated by first boiling it 125

in the presence of sodium sulphide, then allowing the resulting product to cool, and finally distilling the product again in the presence of sulphur.

5 9. The process of concentrating ores by flotation, which comprises adding to a wet ore pulp a quantity of coal tar oil which

has been treated with an alkaline sulphide and sulphur to form a union thereof, and then subjecting the mixture to a froth forming operation.

In testimony whereof, I have subscribed my name.

THOMAS A. JANNEY